

T. M. WHALEN,  
METHOD AND APPARATUS FOR FORMING STEEL INGOTS,  
APPLICATION FILED FEB. 28, 1919.

1,319,500.

Patented Oct. 21, 1919.



*Inventor*  
*Thomas M. Whalen*

*By H. C. Lovell*

*Attorney*

# UNITED STATES PATENT OFFICE.

THOMAS M. WHALEN, OF ERIE, PENNSYLVANIA.

## METHOD AND APPARATUS FOR FORMING STEEL INGOTS.

1,319,500.

Specification of Letters Patent.

Patented Oct. 21, 1919.

Application filed February 28, 1919. Serial No. 279,786.

To all whom it may concern:

Be it known that I, THOMAS M. WHALEN, a citizen of the United States, residing at Erie, in the county of Erie and State of Pennsylvania, have invented new and useful Improvements in Methods and Apparatus for Forming Steel Ingots, of which the following is a specification.

This invention relates to the method and apparatus for forming steel ingots and consists in certain improvements therein as will be hereinafter fully described and pointed out in the claims.

In the forming of steel ingots it is common to place the molten metal in a mold and permit it to cool in the mold. In the cooling of the ingot there are certain faults. The purpose of this invention is to remove to some extent, at least, such faults.

20 The apparatus is illustrated in the accompanying drawings as follows:

The view shows an elevation of the apparatus partly in section.

1 marks the shell of the vacuum case, and 25 2 a cast iron cooling base. The shell at its base is flanged and a gasket 3 is arranged between the flange and the base. The shell is secured to the base by bolts 4. A cover ring 5 is mounted on the top of the shell 30 1, the shell being flanged to receive the ring and a gasket 6 is arranged between the ring and the flange. A cover 7 rests on the ring 5 preferably seated with a tongue and groove joint 8. The cover is secured with 35 eye bolts 9 by means of which it may be clamped to the shell. A mold 10 is arranged in the vacuum case. The mold is provided with a removable bottom 11 and the ingot metal 13 is indicated in the mold 40 45 by dotted lines. A cooling coil 12 is arranged in the base 2 so that the heat may be taken from the metal 13 in the mold 10 and dissipated through a medium such as air or water being caused to flow through said cooling coil 12.

A vacuum pump 14 is connected by a pipe 15 with the vacuum case. The pipe 15 is provided with a valve 16 by which the communication with the case may be closed.

50 A controlling valve 17 is arranged on the cover by means of which the degree of vacuum may be varied. In carrying out my method the molten metal is poured into the mold in the usual manner, the mold 55 having been previously arranged in the vacuum case as shown. The cover is then

put in place so that the case is sealed and the air is exhausted from the case to a greater or less degree as desired.

The inclosure of the mold within the 60 case, thus forming what might be termed a dead air space, would in itself form to some extent an insulation around the mold and consequently temper the cooling action so that a portion of the cooling action 65 at least would take place from the bottom. By exhausting the air from the case the mold is more or less perfectly insulated depending on the degree to which the vacuum is extended. With an exhaustion of the air 70 an almost perfect insulation is provided around the mold and consequently the cooling takes place almost, if not entirely, from the bottom. Consequently the cooling is progressive and the top of the metal 75 remains molten for a longer period and thus accommodates itself to the shrinkage. In this way the usual faults are largely, if not entirely, eliminated.

Further the exhaustion of the air makes 80 the space in which the metal is placed practically inert and, therefore, the deleterious chemical changes are obviated. This is particularly true with some alloys.

It may be desirable to provide the ob- 85 servation openings 18 in the case, these openings being sealed by some transparent material.

What I claim as new is:

1. The method of forming steel ingots 90 which consists in placing molten steel in a mold; insulating a portion of the mold; and cooling the steel from that portion of the mold not insulated.

2. The method of forming steel ingots 95 which consists in retarding by insulation the cooling of a column of molten steel; and cooling the same from the bottom of the column.

3. The method of forming steel ingots 100 which consists in placing a mold containing molten metal in a space insulated from the surrounding air; and cooling the metal from the bottom.

4. The method of forming steel ingots 105 which consists in placing molten steel in a mold; placing this mold in a space insulated by a partial vacuum from the surrounding air; and cooling the metal progressively by dissipating the heat from one part of the 110 metal.

5. The method of forming steel ingots

which consists in placing molten metal in a mold; inclosing the mold in a space made more nearly inert than atmospheric air; and cooling the metal in said space.

5 6. The method of forming steel ingots which consists in placing molten metal in a mold; inclosing the mold in a space made more nearly inert than atmospheric air by the formation of a partial vacuum; and 10 cooling the metal in said space.

7. The method of forming steel ingots which consists in placing molten steel in a mold; inclosing the mold in a space; insulating the mold from the surrounding 15 atmosphere; rendering the same more nearly inert than atmospheric air; and cooling the steel from the bottom.

8. In an apparatus for forming steel

ingots, the combination of a mold; a vacuum case in which the mold is placed; means for 20 exhausting the air from the case; and means for cooling the bottom of the mold.

9. In an apparatus for forming steel ingots, the combination of a mold; a vacuum case in which the mold is placed; means 25 for exhausting the air from the case; means for cooling the bottom of the mold; and means for controlling the degree of vacuum.

10. In an apparatus for forming steel ingots, the combination of a mold; an insulating case in which the mold is placed; and means for cooling the bottom of the mold. 30

In testimony whereof I have hereunto set my hand.

THOMAS M. WHALEN.